

J. C. FOX.

METAL ROLLING.

APPLICATION FILED JULY 24, 1912.

1,147,713.

Patented July 27, 1915.



Fig. 1.



Fig. 2.

Fig. 5.

Fig. 4.

Fig. 3.

Fig. 6.



INVENTOR.

John C. Fox,

by Geo. E. Thackray,  
his ATTORNEY.

WITNESSES,  
Elmer Seavey.  
Jas. E. Williamson.

# UNITED STATES PATENT OFFICE.

JOHN C. FOX, OF WESTMONT BOROUGH, PENNSYLVANIA, ASSIGNOR TO CAMBRIA STEEL COMPANY, A CORPORATION OF PENNSYLVANIA.

## METAL-ROLLING.

1,147,713.

Specification of Letters Patent. Patented July 27, 1915.

Application filed July 24, 1912. Serial No. 711,266.

*To all whom it may concern:*

Be it known that I, JOHN C. Fox, a citizen of the United States, residing in the borough of Westmont, in the county of Cambria and 5 State of Pennsylvania, have invented certain new and useful Improvements in Metal-Rolling; and I do hereby declare the following to be a full, clear, and exact description of the invention, such as will enable others 10 skilled in the art to which it appertains to make and use the same.

My invention relates generally to metal rolling and more particularly to reducing and forming hot metal ingots, blooms, billets, bars or other shapes by a continuous 15 process and apparatus whereby the said metal is operated upon successively by a series of rolls which are preferably placed with the grooves or passes thereof substantially in line, and so spaced as to operate on 20 different parts of the metal at the same time.

Although my invention relates to any shapes of metal, I will, for the sake of simplicity of description and ease of illustration, 25 confine these to the application of my invention in connection with rolling small billets, or approximately square bars with rounded corners, from larger sections commercially known as blooms, and in order to 30 further simplify the description herein, I will generally refer to the various sections as bars.

Heretofore in this art it has been the general belief that it sufficed to overlook, and 35 consequently it became the practice to neglect the finer and appropriate niceties of the design and to somewhat crudely proportion the rolling mill and the successive grooves or passes of the rolls thereof, so that 40 the amount of material delivered from one pass to the next pass, and the amount which is received and transmitted by said next pass, will be only approximately equal to each other. These amounts are dependent, 45 among other things, upon the relative cross sectional areas of said passes and the speed ratios of the respective pairs of grooves in the rolls. This practice resulted in inequalities of operation, whereby, at times, considerably 50 more material was delivered from one pass than from the succeeding pass, thereby causing an overfill and deformation of the material in the latter; or otherwise, more material was drawn by the succeeding 55 pass from the preceding pass, thereby caus-

ing a tension in the bar between said passes and producing a wire-drawing action between successive pairs of rolls, in addition to the reducing action of the roll passes. By careful study and experimentation I have 60 discovered that rolls designed in this latter manner, that is, with a tension or drawing action between the passes, may operate approximately correctly when the grooves of the various tandem continuous series of passes 65 are filled with a bar extending through a number of said passes, but when the rear end of the bar issued from one of such passes, the tension and drawing action was at once relieved in that portion of the bar, thereby 70 causing an overfill, fin or deformation of said bar in the next pass.

My invention consists generally in the arrangement and proportion of a series of continuous roll passes in a series of rolls, each 75 succeeding pair of which has an increased speed, all in such a way as to obviate the difficulties mentioned and to thereby regularly produce bars of full and proper section, but without fins, seams or other imperfections 80 caused by inaccurate proportions and design of the rolls and passes therein.

In order to properly proportion the roll passes for a given amount of reduction of area of the bar which passes there-through, 85 I have discovered that due and careful regard must be had to what I call the "effective diameter" of the roll. By "effective diameter" I mean that diameter passing through the axis of the roll at substantially 90 right angles thereto, the ends of which diameter travel at approximately the same speed as the bar after it has issued from the forming pass, and at the same time when it has acquired regularity of longitudinal 95 movement of translation given to it by frictional contact with the surfaces of the roll passes. As explained herein, I have discovered that this effective diameter is not necessarily that diameter which corresponds 100 to the cylindrical surface of contact of the roll in the case of an approximately flat, square or rectangular bar, but is a greater diameter, and in the case of a diamond-shaped bar this effective diameter does not 105 correspond with that of the bottom of the groove, but is considerably greater. Further details of this will hereinafter appear.

Having thus given a general description of my invention, I will now, in order to make 110

the matter more clear, refer to the accompanying sheet of drawings on which like characters of reference refer to like parts.

Figure 1 is a diagrammatic end elevation 5 of a series of twelve stands of two-high rolls, which operate successively upon the bar as shown. Fig. 2 represents the series of passes or grooves formed in the rolls shown in Fig. 1, the grooves of each set 10 being drawn as cross sections directly below the rolls but on an enlarged scale, so that their forms and proportions may be readily seen. Fig. 3 indicates approximately rectangular bars incorrectly rolled by previous 15 methods, the first one having a fin and the succeeding one having a seam caused thereby; while Fig. 4 represents bars of similar general shapes rolled by my improved method to proper proportions without fins, 20 seams or deformations. Fig. 5 represents diamond and square bars rolled by my method from the last passes Nos. 11 and 12, showing the correct form without fins, seams or deformations; while Fig. 6 shows bars of 25 similar sections rolled improperly by other methods, with fins, seams and imperfections caused thereby.

Referring now to the detailed characters of reference on the drawings, the different 30 pairs of rolls Nos. 1, 2, 3 and 4 represent the preliminary rolls which are preferably of larger diameters than the succeeding ones, in order to contain passes therein of size sufficient to accommodate the large bloom or 35 billet with which my rolling operation begins. The pairs of rolls 5, 6, 7, 8, 9, 10, 11 and 12 are of smaller diameter and represent in the order of their numbers the succession of pairs of rolls between which the bar 40 passes continuously.

B represents the bloom or bar as it enters between the pair of rolls 1, and B' represents the front end of the finished bar or billet as it issues from the last pair of 45 rolls 12.

Between rolls 1 and 2 a twisting arrangement is used (not shown) in order to give the bar a quarter turn before entering the pair of rolls 2, and similar twistings are used 50 between the pairs of rolls 3 and 4 and 5 and 6. These rolls 1 to 6 inclusive contain grooves known as box passes. After leaving the pass in the rolls 6, the bar is formed into what is known as an oval or diamond-shape 55 in rolls 7, and between the pairs of rolls 6 and 7 I provide a twisting guide which gives the bar an eighth of a turn. Similar twisting guides provided with an eighth turn are arranged between rolls 7 and 8, 9 and 10 and 60 11 and 12, in order to quickly reduce the diamond or oval into the approximately square form as indicated. This arrangement of twists is shown to complete the illustration, but is not essential to my invention, as 65 my method and apparatus can be used with-

out twistings in cases where preferable, as will be readily understood by those skilled in the art of metal rolling.

The cross sections of the roll passes, as I have designed them in accordance with my 70 invention, are indicated successively as  $a^1$  to  $a^{12}$  inclusive, in Fig. 2, and for convenience of reference each of these drawings is placed directly below the pair of rolls to which it applies. It will be noted that approximately 75 one-half of each pass is formed in the top roll and the other half is formed in the bottom roll with partings, or slight distances between the collars, adjoining the passes, all as indicated in Fig. 2. The speed of longitudinal movement of the bar increases step by step successively as it issues from each of the roll passes, the initial movement thereof being slow and the final delivery being comparatively very rapid. The collars of 80 the rolls or those portions adjoining the sides of the passes are indicated as  $g$ ,  $g$ ,  $g$  and the partings or diametral distances between said collars are indicated as  $e$ ,  $e$ ,  $e$ .

Referring now to the difficulties heretofore mentioned in connection with improperly designed roll passes:— $b^6$  indicates a bar which would be formed, for example, in the pair of rolls 5 under these conditions, 90 that is, with tension existing between the pair of rolls 4 and the pair of rolls 5. The reason for this is that as the bar travels in the direction of the arrow between the rolls 4 and 5, the grooves have been so designed 95 in connection with the speed ratios of said rolls that a tension or pulling action exists in the bar between said pair of rolls, which reduces its diameter as it proceeds between them. When, however, the end of the bar passes out from between the pair of rolls 4, 100 this tension and wire-drawing action no longer exists, so that the grooves in the rolls 5 receive more metal than they can properly 105 form and reduce, with the result that the metal extrudes between the roll partings 110 forming fins as indicated in  $f^6$ . When the bar  $b^6$  is given a quarter turn and rolled by the pair of rolls 6, these fins are pressed down into the body thereof and form seams or imperfections as indicated at  $s^6$  in the bar  $b^6$ .

Section  $b^{11}$  in Fig. 6 represents a section 115 of a bar produced in the pair of rolls 11 by an improper method due to the fact that the grooves in the rolls 10 and 11 are so proportioned with respect to their speed ratios, 120 that a tension exists in the bar between the pair of rolls 10 and the pair of rolls 11, or in a previous pair, causing a fin  $f^{11}$  in the bar  $b^{11}$  for the same reasons as those previously mentioned. Similarly the seams  $s^{12}$  125 are formed in the succeeding bar  $b^{12}$  which causes an imperfection in the finished product. In case a tension exists between the pair of rolls 11 and 12, the fins  $f^{12}$  will ap- 130

pear on the last end of finished bar  $c^{12}$ , as it issues from the last pair of rolls 12, or in case this happens in connection with a fin such as  $f^{11}$  on the previous bar  $b^{11}$ , a fin  $f^{12}$  and a seam  $s^{12}$  will appear on the finished bar  $d^{12}$ , causing a double imperfection. On the other hand my rolls are designed in such a way that no appreciable or deforming tension can exist between the successive pairs 5 of rolls such as between the pairs 4 and 5, so that when the bar issues from the pair of rolls 4, the same amount of material in the last end of the bar is furnished to the pair of rolls 5 as before. This being the 10 case, there is no excess of metal delivered to the pair of rolls 5 and the operation proceeds properly and uniformly with the result of producing good sections such as  $a^5$  and  $a^6$ . Similarly, I produce by means of 15 my invention, sections such as  $a^{11}$  and  $a^{12}$ , free from the imperfections noted.

Although the foregoing is plain to those persons familiar with continuous metal rolling, in order to make this matter more 20 clearly understood, it might be stated in approximately the form as follows:—Let  $D$ = the effective diameters of the roll passes, that is, the diameter of the circle passing through the cross section of said roll pass in 25 a plane at right angles to the roll axes, the center of one roll axis being the center of the said circle, the circumference of the circle passing through that point of the cross section of the bar which corresponds with 30 its forward lineal velocity as given to it by the frictional contact of the bottom or the sides of the roll pass or a combination thereof, as may be. Let  $\pi$ =the usual ratio of the circumference of a circle to its diameter, 35 viz.:—3.14159+. Let  $A$ =the areas of the cross section of the bars formed in the pairs of rolls in question. Let  $R$ =the speed ratios of the rolls, that is, the number of revolutions per unit of time of any pair of rolls 40 as compared with the first pair, which latter for convenience of calculation may be assumed as unity. Then, in order to properly design the rolls in accordance with my invention, the product of  $D$  by  $\pi$  by  $A$  by  $R$  45 should, for each pair of rolls, be very slightly greater than that of the corresponding product for the succeeding pair of rolls, thus avoiding tension of the bar between the successive pairs of rolls, thereby obviating 50 the consequent difficulties connected with said tension, as herein described.

The effective diameter of the rolls varies considerably with the shape of the groove and somewhat with the heat or plasticity of 55 the material passing therethrough. Generally speaking, however, I consider that the effective diameter of a box pass such as  $a^2$ , is the diameter of a circle located as heretofore described, the circumference of which 60 passes through a point about one-fourth the

distance from that surface of the bar which is in frictional contact with the surface of the roll, toward the center of the cross section of the bar. The effective diameter of the diamond or gothic square sections which 70 are rolled diagonally, as indicated in passes  $a^7$  to  $a^{12}$  inclusive, is that of a similar circle passing through a point about 70% or three-fourths the distance from the lower rounded corner of the said bar and the center of said 75 bar, and these are the figures which I prefer to use in proportioning rolls in the manner heretofore described for the purposes mentioned in accordance with my invention.

To explain the matter in still another way, 80 viz.:—One of the essential points on which my invention is based in order to prevent fins, seams and deformations in continuous rolling, is to deliver a very slight excess of material from one pass to the next, thereby 85 preventing tension or drawing action between one pass and the next. For example:—If there is tension between the pair of rolls 1 and the pair of rolls 2 then when the piece leaves the pair of rolls 1, this tension 90 at once ceases and the pair of rolls 2 is over-filled, making a fin, which fin is rolled down in No. 3 rolls, causing a seam. Many attempts have been made to overcome this 95 difficulty by rolling-mill men, but until my discovery and invention, these prior attempts have not been successful.

In practising my invention I may make detailed calculations showing the proportions between the various roll passes, the 100 speed ratios and other elements thereof, to insure the absence of appreciable or deformatory tension in the bar between the successive passes sufficient to prevent the difficulties mentioned as inherent in prior practice, 105 but as all these are subject to slight changes and variations within the scope of my invention, any further details are considered unnecessary, and particularly so as the descriptions herein will fully explain the matter to those skilled in this art.

Although I have shown and described my improvements in considerable detail, I do not wish to be limited to the exact and specific details shown and described, but may 115 use such substitutions, modifications or equivalents thereof, as are embraced within the scope of my invention as pointed out in the claims.

Having thus described my invention, what 120 I claim and desire to secure by Letters Patent is:—

1. The method of continuous rolling, which consists in delivering a slight excess of material from one roll pass directly into 125 the next, whereby tension is avoided in the bar between contiguous passes, thereby preventing fins, seams or deformations in said bar.

2. The method of metal rolling which con- 130

sists in simultaneously reducing a bar in a plurality of continuous alined passes, and in delivering a slight excess of bar material directly from one pass into the next, where-  
5 by an appreciable or deformatory tension is avoided in the bar between contiguous passes.

3. In a metal rolling mill, a plurality of alined roll passes adapted to simultaneously  
10 reduce a bar passed therethrough, the cross sectional area of a preceding pass and the effective diameter of the same being so adjusted as to deliver in a given time a slight excess of material from said pass directly  
15 into the next succeeding pass, as compared with the amount of material delivered by said succeeding pass.

4. In a continuous metal rolling-mill of

the class described, a pair of alined roll passes adapted to simultaneously reduce a bar passed therethrough, the cross sectional areas and the effective diameters of said passes being so adjusted as to deliver a slight excess of bar material from one pass directly into the next pass in a given time, 25 thus avoiding appreciable or deformatory tension of the bar between said passes, thereby preventing fins, seams or deformations in said bar.

In testimony whereof I hereto affix my 30  
signature in the presence of two witnesses.

JOHN C. FOX.

Witnesses:

J. F. GROGAN,  
ROBT. A. BEERS.